

Patented Apr. 10, 1923.

1,451,462

## UNITED STATES PATENT OFFICE.

ABRAHAM ALBERT KLEIN AND MILTON F. BEECHER, OF WORCESTER, MASSACHUSETTS, ASSIGNORS TO NORTON COMPANY, OF WORCESTER, MASSACHUSETTS, A CORPORATION OF MASSACHUSETTS.

## NONSLIP TILE.

No Drawing.

Application filed November 11, 1920. Serial No. 423,423.

To all whom it may concern:

Be it known that we, ABRAHAM ALBERT KLEIN and MILTON F. BEECHER, citizens of the United States of America, residing at 5 Worcester, in the county of Worcester and State of Massachusetts, have invented certain new and useful Improvements in Non-slip Tiles, of which the following is a full, clear, and exact specification.

10 This invention relates to safety treads and more particularly to tiles and terrazzo adapted for use on stairs, ramps, platforms and other places where pedestrian travel is heavy and there is large danger of accidents 15 due to slipping thereon.

As disclosed in the patent to Jeppson and Dietz No. 1,292,953 of January 20, 1919, it has been proposed to make a non-slip surfacing of extremely hard materials, such as 20 crystalline alumina and silicon carbide, bonded by ceramic materials fused at a high temperature, approximately 1300° C. We have found that there is a tendency for such extremely hard and durable tiles to show some decrease in anti-slipping characteristics after prolonged usage under certain types of traffic conditions. This is considered to be due in part to the pores becoming loaded with foreign bodies. Also, the abrasive grains and bond tend to wear down to a smooth surface and the tread does not retain its maximum safety properties or possess the capacity for self renewal to a sufficient extent. In such cases, the grains are apparently too hard and too firmly bonded together, so that the tread cannot disintegrate to the slight extent required to maintain an abrading surface. At the same time, the grains must be bonded by a material, while softer and somewhat brittle, which is tough enough to hold the grains in place until their period of efficiency is past.

As a further consideration, the electric furnace products heretofore utilized for such treads have been expensive and have required high temperature methods for bonding them into tiles of sufficient strength and durability to resist premature disintegration by traffic usage; hence the use of safety treads 50 has not been promoted to the fullest extent because of the initial cost of the tiles.

It is accordingly an object of our inven-

tion to overcome such objections by making a safety tile of abrasive materials softer than alumina which will satisfy the requirements of safety engineers for light traffic conditions and by bonding such abrasive grains with suitable ceramic substances which are tough, durable and capable of uniting with the grains to form a long lived tile and yet will permit renewal or maintenance of the anti-slipping properties of the tile surface as is required for a satisfactory tread.

Another object of this invention is to utilize the natural abrasive materials, ranging in hardness from 7 to 9 on Mohs' scale, which possess desirable characteristics adapting them for non-slip purposes, and to employ those minerals to this end which are too fusible to be used in accordance with the former high temperature method of making ceramic tiles.

A further object is to simplify the procedure and lessen the expense of bonding granules of various types of anti-slipping material and yet obtain an article which is substantially weatherproof and highly resistant to disruption by pedestrian abrasions. Further objects will be apparent in the following disclosure.

In accordance with this invention, we propose to utilize materials, having a hardness of from 7 to 9 on Mohs' scale, which have tough crystalline structures and are not easily broken and which have high abrasive or non-slip qualities, and to bond grains of such materials together into a wear-resisting, anti-slipping article by means of softer ceramic bonds which are able to hold the grains in place for a long period under the ordinary usage of pedestrian traffic. The various abrasive materials suitable for this purpose, which are harder than quartz, include the various spinel abrasives and particularly that spinel known as magnesium aluminate, the garnets, such as calcium aluminum silicate, beryl and the low grade emerys, such as Peekskill emery, which contains a high percentage of iron oxide and may contain a large amount of the iron spinel, hercynite.

In order to unite these grains into an integral mass of the proper density and

120. Al 3

porosity, as well as tensile strength and ability to withstand the shocks and strains of pedestrian wear, we propose to utilize various ceramic bonds, such as clay materials vitrifying to a glassy or a porcelanic condition for those materials which do not soften or change at the temperature of vitrification of the bond. The various low fusing silicates, such as sodium silicate, are available where it is required that the bonds be fired at low temperatures, so as not to affect the abrasive or non-slip characteristics of the tile. For such materials as the ordinary magnesium aluminate spinel, we utilize clay mixtures adapted to burn to a glassy nature, or bonds which are formed by combining the more refractory clays with various fluxes, such as soda, magnesia, calcium oxide, lead oxide, barium oxide, etc., thus producing complex silicates having a glassy fracture and the qualities of great durability and tenacity to hold the grains together. As a specific example of a ceramic bond suitable for use with magnesium aluminate spinel, the following ingredients may be used in the proportions specified:

|               |                    |
|---------------|--------------------|
| Feldspar      | 22 parts by weight |
| Ball clay     | 10 " " "           |
| Slip clay     | 13 " " "           |
| Spinel grains | 55 " " "           |

A plastic mixture of these materials and water is formed into a tile shape, dried and then fired in a ceramic kiln, in accordance with the usual practice. The firing treatment may involve heating the ware at approximately cone 12 for several days and then slowly cooling, this procedure resulting in the formation of a glassy or vitreous mass intimately uniting the spinel granules into a unitary but porous structure in which the anti-slipping grains constitute the wear-receiving part of the surface and preferably the major portion by volume of the tile.

We have also found that low fusing abrasive materials may be employed and yet a tile of high bond strength and tough wear-resisting characteristics obtained. This is accomplished by employing a bond which is capable of uniting integrally with the grains below the fusion temperature of the granular material and preferably reacting with or dissolving the surface layer of the grain to form a strong intermediate layer. Garnet and beryl are examples of this class of materials. In order to bond garnet and beryl, which melt or become deleteriously affected at a temperature below that of the ordinary ceramic operation as above described, we propose to use various silicate mixtures capable of forming a glassy bond at a low temperature.

As a specific example of a tile of beryl united by a durable silicate bond, which is substantially insoluble, the following for-

mula and procedure may be adopted. A dry mixture may be made up of:

|                     |                    |
|---------------------|--------------------|
| Beryl               | 80 parts by weight |
| Dry sodium silicate | 7 " " "            |
| Zinc oxide          | 1 part " " 70      |
| Albany slip clay    | 2 parts " "        |

To this dry mixture may be added 9 parts of wet sodium silicate having a specific gravity of about 60° D. The wet silicate is thoroughly mixed with the dry ingredients in a kneading machine. The mixture is then of the proper consistency for shaping, as by tamping or dry pressing. After the tile has been shaped, it may be dried in a steam box for a few hours at about 140° C. and then fired to a vitrified condition by heating to approximately 900° C. for several hours' time. Various bond ingredients may be substituted for those above specified, as is well known in the ceramic art.

It has been found that the utility of a tile of this type as a safety tread depends largely upon two main factors, the sizes of the grains employed and the porosity of the tile. It is desirable that the surface of the tile contain a number of large grains of about 30 mesh in order to afford a safe foothold and that these be combined with other grain sizes which will reduce the porosity of the tile to a safe minimum and aid the bond in strengthening the tile. In the formula above specified for a spinel tile the abrasive is made up of 50% of 30 mesh grain, 30% of 60 mesh and 20% of 120 mesh. The porosity of this tile as determined by water absorption is about 8 to 10% by volume. We find it desirable to combine such grain sizes as to give a porosity of from 5 to 20%. In this way we keep the grains largely isolated so that the bond between the grains will not prevent the abrasive material from getting a good hold on footgear. This porosity arises from the fact that in the firing operation the ceramic bond shrinks into a dense vitreous mass in the form of walls and separated posts which tie together the adjacent surfaces of the grains.

Due to a slight reaction between the bond and certain of the available grain materials, such, for example, as is found in the magnesium aluminate spinel tending to react with the fused clays to form various complex compounds, the materials are in such instances bonded into a substantially integral mass having a tenacious and durable structure which will withstand pedestrian wear for an indefinite time. It is our intention to utilize in so far as possible such combinations of bonding materials for each type of abrasive grain chosen that an integral union will be had, this characteristic of course being modified or determined by the physical properties of the abrasive employed. We therefore are able to obtain

sufficient tile strength, although using a low fusing abrasive material, by selecting a ceramic bond which is fusible at a still lower temperature and preferably is capable of

- 5 reacting to some extent with the surface portions of the grains to form an intermediate layer of the grain material dissolved in or united with the bond material. By employing grains and bond which have less difference in hardness than found in the tiles here-  
10 tofore proposed, we provide an article which is adapted for light traffic conditions, where the bond itself should receive some wear and occasionally break away to expose fresh and
- 15 sharp grains on the surface, and so avoid detrimental loading of the tile pores and glazing of the surface.

Having described our invention, what we claim as new and desire to secure by Letters

20 Patent is:

- 1. A non-slip tile comprising wear-resisting abrasive granular material of a hardness between quartz and crystalline alumina and a ceramic bonding material integrally united  
25 by heat into an abrasive, wear-resisting and substantially integral mass in which the granular material constitutes a substantial proportion of the surface of the tile and the bond is capable of permitting renewal of the  
30 safety characteristics of the tread surface.
- 2. A non-slip tile comprising abrasive granular material of a hardness between 7 and 9 on Mohs' scale and a high burned ceramic bonding material integrally united  
35 into a non-slip, wear-resisting mass in which the granular material constitutes the major portion of the volume of the tile.
- 3. A non-slip tile comprising wear-resisting, crystalline anti-slipping granular material of a hardness between quartz and

alumina bonded together by an alkaline silicate bond into a porous mass, in which the granular material receives the major portion of the tread wear.

4. A non-slip tile comprising abrasive granules of material having a hardness between quartz and alumina and a ceramic bond adapted to resist pedestrian wear which may be matured by heat at a temperature below the fusion point of said granular material, the major portion of said granules being between 30 and 120 mesh in size, and the bonded mass having an absorption between 5% and 20%.

5. A non-slip tile comprising wear-resisting, anti-slipping granular material having a hardness greater than 7 on Mohs' scale bonded together by a vitrified alkaline silicate bond.

6. A non-slip tile comprising granular material of a hardness between 7 and 9 on Mohs' scale which softens below 1200° C., bonded by a vitrified alkaline silicate bond.

7. A non-slip tile comprising granular beryl bonded by a vitrified clay and alkali silicate bond.

8. A non-slip tile comprising abrasive material, which has a hardness between quartz and crystalline alumina and is fusible below 1200° C., and a high burned insoluble bond including sodium silicate, said abrasive material constituting the major portion of the tread surface and being between 30 and 120 screen mesh in size and the tile having a water absorption of 5 to 20% by volume.

Signed at Worcester, Massachusetts, this 5th day of Nov. 1920.

A. ALBERT KLEIN.  
MILTON F. BEECHER.